

## UNITED STATES PATENT OFFICE

GEORGE F. DORAN, OF WORCESTER, MASSACHUSETTS

61

## SHAVING SOAP

No Drawing.

Application filed December 29, 1925. Serial No. 78,233.

This invention relates to soaps and particularly to a soap especially adapted for shaving or shampoo.

Among the objects of the invention are to provide a soap of sufficient hardness to adapt it to be manufactured in the form of a bar, dry stick, or powder, while at the same time possessing the capacity for forming a profuse lather.

10 A further object of the invention is the provision of a shaving soap including a specific ingredient for softening the beard.

Other objects of the invention will appear as the following description of a preferred embodiment thereof proceeds.

Ordinarily hard soap is made by the saponification of tallow or other animal fat by means of an alkali such as caustic soda. The tallow contains two fatty substances, one of which, stearin ( $C_{57}H_{110}O_6$ ) is solid, and the other, olein ( $C_{57}H_{104}O_6$ ) liquids, the quantity of stearin being about thrice that of olein. The presence of this proportion of olein in the soap detracts from its degree of hardness 25 to an extent which renders it inadapted for pulverization, while the olein itself is of only fair capacity as a lather producer, as is also the stearin itself so that the average tallow soap is not characterized to a marked degree 30 by those qualities which go to make an ideal shaving soap.

By my invention the use of tallow as a base is avoided, the most desirable constituent of the tallow, that is to say the stearin being used in the form of stearic acid. The stearic acid used in this soap is what is known as "triple pressed", the same heretofore, when used in a predominating quantity, being unfit for shaving soap due to the impossibility 40 of producing the moist lather necessary in shaving. However, by mixing it as herein-after set forth with approximately one-third the quantity of cocoa-nut oil, with three-third of stearic acid properly proportioned 45 with lye, it has been found in practice that the stearic acid will produce a hard soap, that is, a soap very solid in texture, and which can be molded into cakes or sticks or comminuted to produce a very fine soap for 50 shaving, and will produce a lather especially

desirable for this purpose. Through avoidance of the use of olein, the hardness of the soap is greatly enhanced so that it may be formed into a dry stick of economical hardness, or readily comminuted into a pulverulent material.

In place of the olein I substitute a vegetable oil such as cocoa-nut oil which contains a vegetable fat known as trilaurin ( $C_{39}H_{74}O_6$ ), which does not diminish the hardness of the soap and at the same time possesses when saponified a high degree of surface tension in aqueous solution, forming a profuse lather.

In carrying out the step of saponification 65 I may use various proportions of stearic acid and cocoa-nut oil. For instance seven and one-half pounds of stearic acid may be melted with two and one-half pounds of cocoa-nut oil to which four pounds of lye are added. 70 In making a soap according to the present invention I have found that a lye containing equal proportions by weight of sodium hydroxide and potassium hydroxide gives good results, although the exact constituency of the 75 lye is not an essential feature of the invention.

In making my soap, I first heat the stearic acid and cocoa oil to 160° Fahrenheit and add the glycerine, if this ingredient is to be used. 80 Then I add the lye solution composed of potash and soda with the two lbs. water. This lye solution is cooled down to 60° Fahrenheit. Stir as the lye is added. It saponifies immediately and heats up. Mix for ten minutes, 85 at which time the whole is saponified.

When the saponification is completed other desirable ingredients such as glycerine, water and perfume may be incorporated and I also add a mild alkali such as borax in the proportion of two ounces to the weights of the other ingredients above mentioned. This alkali is for the specific purpose of softening the beard. The soap is then framed as usual and cut into bars, or if to be used in powder form it is permitted to harden and then pulverized.

The borax used is a very mild alkali, and in practice it has been found where used as a 5% part of the soap of a solution, that it has a

tendency to soften the beard without injury to the skin; in fact, to the most delicate of skins.

While I have in the above disclosure described a soap eminently adapted for shaving or shampoo, it is to be understood that my invention is by no means limited to a shaving soap but will be found equally good for most detergative purposes.

10 Having described my invention what I claim as new and desire to secure by Letters Patent, is:—

15 A shaving soap formed by mixing together the following ingredients, triple pressed stearin acid approximately 53.6%, cocoanut oil approximately 17.8%, sodium hydroxide approximately 14.3%, potassium hydroxide approximately 14.3% and borax approximately .5%.

20 In testimony whereof I have hereunto set my hand.

GEORGE F. DORAN.

25

30

35

40

45

50

55

60

65